

## UNITED STATES PATENT OFFICE

2,111,800

## PROCESS OF TANNING

Theodore F. Oberlander, Elkland, Pa.

No Drawing. Application June 27, 1934,  
Serial No. 732,624

## 4 Claims. (Cl. 149—5)

This invention relates to the treatment of hides and leather. It is an object of this invention to produce a leather with an improved quality and durability. It is a further object to provide a process which will control the acid content of the leather and thereby increase its length of life and serviceability. It is a further object to produce a leather which will be of a uniform quality with a minimum of expense and difficulty. It is a further object to devise a process for the production of leather which will be simple to operate and which will be effective and reliable in its results.

In the treatment of leather the raw hide, after the hair and flesh are removed, is treated with a tanning solution to convert the hide into leather. It may then be washed and bleached either by the use of soda ash or other bleaching agent, thereafter it may be tumbled in a drum with a filler solution, molasses, Epsom salts or the like. The leather may then, if desired, be again soaked in a cellulose sulphate or tanning material and again treated with fillers, sugar, Epsom salts and oil. For many purposes this second step may be omitted. After the leather is treated it may be conditioned so that it may be compressed by a press or rolling machine and it may be further bleached if desired by dipping in a sponge or dipping compound.

The finished leather produced by the above process has a serious drawback in that it is apt to have an unduly high acid content which makes it unsuitable for many purposes and which is destructive of its durability. This acidity may be due to the acids of the tanning solution or it may be due to the acids used in bleaching and it may run as high as two percent of free mineral acid.

In accordance with this invention it has been found that the effect of these acids insofar as they produce an acidity in the finished leather may be substantially neutralized by the use of magnesium carbonate in solution either in the presence of the tanning materials or after the last acid bath without in any manner destroying or counteracting the essential purposes of the tanning acids in the formation of the leather.

A typical method of using it will be to make up a mixture of the following approximate proportions, 50% powdered tanning or filling extract, 8% oxalic acid, 1% borax, 10% Glauber salts, 8% magnesium carbonate, 5% kaolin, 1% sodium acid sulphate or potassium acid sulphate and 17% sodium chloride.

When used in this manner the magnesium carbonate serves to control the acidity in the finished

leather without destroying the beneficial effect of the other ingredients.

Another typical method is to use a desired amount of magnesium carbonate in the oil wheel during the process of adding oil, sugar or Epsom salts to the leather.

In any case the amount of magnesium carbonate to be added to the solutions will depend on the solution used and the character of the leather to be treated and produced, and the most desirable proportion can most readily be determined by the results.

Leather made in accordance with this process may be kept with a substantially uniform content, for example, between 0.3% and 0.7% of 15

The use of other carbonates than magnesium carbonate is not so effective, some of such carbonates for example as sodium carbonate when used in appreciable quantity tends to prevent the functioning of the tanning process and other carbonates such as barium carbonate are too inert to be of value.

Since certain changes may be made in the above construction and different embodiments of the invention could be made without departing from the scope thereof, it is intended that all matter contained in the above description shall be interpreted as illustrative and not in a limiting sense.

It is also to be understood that the following claims are intended to cover all of the generic and specific features of the invention herein described, and all statements of the scope of the invention which, as a matter of language, might be said to fall between said claims.

Having described my invention, what I claim as new and desire to secure by Letters Patent is:—

1. The process of tanning which comprises 40 treating the hides with a vegetable tanning solution and subsequently neutralizing the acidity with magnesium carbonate.

2. The process of tanning which comprises 45 treating the hides with magnesium carbonate in conjunction with vegetable acid materials to control the acidity of the finished hide.

3. The process of treating leather which consists in subjecting vegetable tanned hides to the action of magnesium carbonate in solution to 50 limit the final acidity.

4. The process of treating leather which consists in subjecting it to a vegetable acid tanning solution in the presence of magnesium carbonate.